

## UNITED STATES PATENT OFFICE.

GOODWIN H. HOWE, OF SCHENECTADY, NEW YORK, ASSIGNOR TO GENERAL ELECTRIC COMPANY, A CORPORATION OF NEW YORK

## TREATMENT OF METALS.

No Drawing.

Application filed April 1, 1925. Serial No. 19,999.

My invention relates to the art of treating metal so as to protect them against the effects of oxidation and other corrosive agencies, and has for its object the production 5 of a coating upon a metal normally subject to corrosive action or a condition within the metal such that it is capable of withstanding the oxidizing and corrosive influence without harmful effect.

10 My invention relates more specifically to the treatment of such metals as iron, steel and copper, which readily oxidize at elevated temperature. It is now well known that these metals may be very effectively protected by treating the surface with aluminum so as to cause the aluminum to alloy with the foundation metal. The trade name for this treatment of metal is "calorizing". This fundamental idea is disclosed in a patent 15 to Tycho Van Aller No. 1,155,974 dated October 5, 1915. According to the Van Aller process, the article to be treated is brought into contact with aluminum powder at a proper temperature and under conditions which prevent oxidation of the metallic article, the treatment taking place in a closed oven which slowly rotates. After being thus treated for a proper length of time, which may be about two hours, the article is 20 fired at a temperature of between 700 and 800° C. for 15 or 20 minutes. More recently it has been found that a similar result may be obtained by dipping the article under proper conditions, in molten aluminum and 25 then firing. Examples of this process will be found in patents to Anseleno Ortez #1,409,017, William J. Keep #1,456,274, Christian Dantsizen #1,381,085 and others. These processes, while very satisfactory, are 30 more or less limited in their application to articles of certain shapes and sizes. Obviously, it would be impracticable to treat very large, irregular shaped articles by the Van Aller process and, while it is possible to 35 provide a very large bath of molten aluminum for the dipping process, it will be obvious that there are likewise limitations to this process. Furthermore, the maintenance of a large bath of molten aluminum is 40 expensive and some metals, such as non-ferrous metals, may be injured or even dissolved in such a bath.

It has been realized for quite some time that if the aluminum could be applied as a 45 paint is applied, this field of protection of

metals would be greatly broadened. This would result not only from the wider application by reason of the increased dimensions of the articles which could be treated, but, also because of the decreased cost of operation. Attempts have been made to use the ordinary aluminum paint of commerce and other paints containing aluminum but these have all failed to produce the desired 60 result. One of the reasons for this failure is that these paints all contain solid matter which interferes with the penetration of the aluminum into the article. Furthermore, ordinary aluminum paint affords no protection against oxidation during firing. I have 65 found that in order that the aluminum shall penetrate the article during firing, it is essential that the aluminum shall be in contact with a clean surface and provision should be made to prevent oxidation of the aluminum 70 and, also of the foundation metal while the penetration is taking place during firing. I have also found a way of causing aluminum powder to adhere to the clean surface of the foundation metal under conditions which 75 will permit and cause the aluminum to penetrate. In other words, I have found a way of applying the aluminum in the way paint is applied and in a cold condition and at the same time produce a product which is equal, 80 if not superior, in quality to that produced by the powder and dipping processes above referred to.

In carrying out my invention I employ a mixture of aluminum powder, preferably of 85 the granular form, with a suitable binder. Ordinary commercially pure aluminum may be used, such as 99% pure aluminum. I have found that certain grades of nitrocellulose 90 which are soluble in either amyl acetate or wood alcohol form, when so dissolved, a solution which is admirably adapted for the purpose of acting as a binder for the aluminum powder in applying it to the article. Such a solution is known in commerce under 95 the name pyroxylin. The properties of this solution which make it so desirable for my purpose are as follows: First, it wets and firmly adheres to metals; second, its solvents and thinners evaporate rapidly and leave the nitrocellulose which acts as a binder; third, the nitrocellulose which is left as a binder volatilizes before a temperature is reached 100 which will cause the aluminum to penetrate the foundation metal and leaves only from 105 110

5 to 2% ash, about half of which is silica, which in such small quantities is harmless; fourth, it is non-hydroscopic.

The surface of the article is first thoroughly cleaned either by sand blasting or pickling. A mixture made of aluminum powder and this solution may then be applied in the ordinary way of applying paint. It may be applied with a brush, or by properly thinning with the solution it may be sprayed on. I have even found that a very satisfactory result may be obtained by dipping the article in a bath of this cold mixture. The mixture may also be applied in the form of paste. It might here be noted that the aluminum powder remains in suspension in this solution surprisingly well, although it will probably be desirable to provide means for stirring when the mixture is being used in large quantities. The coating should be made as even as possible and this can be done very easily as the mixture has the property of being very readily spread. When an even and continuous coating has been applied to the article, it is dried. This may be hastened by placing the coated article in an oven for about 15 minutes at a temperature of from 60° C. to 100° C. After drying it will be found that the aluminum is quite firmly adherent, at least it cannot be rubbed off easily, and the article may be handled without injury to the coating. Of course, in this condition it may be injured by contact with a hard object and may even be scratched with the finger nail, but the coating will not be rubbed off by the ordinary contact with the hand. Further coatings may be applied until the desired thickness is obtained.

The article is now fired. This may, if desired, be done in an atmosphere of hydrogen but I have found that with certain materials, such as the ferrous metals, as good results are obtained by firing in the open air. When copper is being treated it is preferable to fire in a hydrogen atmosphere. This brings out one of the chief values of the nitrocellulose solution. It binds together the fine granules of aluminum and, by excluding any appreciable amount of oxygen, allows an uncontaminated alloy to form. In the case of iron the firing is done at 750°-900° C. for about an hour after which the article is removed and left in the open air to cool. Copper should be fired at a temperature of about 800° C. from 5 to 10 minutes after the article has been heated to that temperature. With iron lower temperatures may be used if the time of firing is increased, and this is true to some extent with copper.

The articles thus treated have a protective coating which in some respects is superior to that produced by the powder and

hot dipping process. The coating seems to be even more firmly adherent, at least it will withstand a surprising amount of bending. Furthermore, the coating has a very definite and firm outline, that is to say, it resists oxidation from an adjacent unprotected area, the result of which is that an unprotected area does not grow and effect protective areas as has been found to be the case with the other methods of treatment referred to. This point is illustrated by the following experiment. A paste was made of the proper consistency to form drops with good outline detail. drops of the material were placed upon several  $\frac{1}{8}$ " thick test pieces of iron and fired in air at 750°-900° C. The test pieces were then placed in a furnace at about 1000° C. and run for three days. Morning and night they were removed from the furnace, allowed to cool and the loose scale removed. At the end of three days the pieces were burned to destruction with the exception of the spots covered by the drops which remained intact with the outlines still well defined.

The following test which demonstrated how firmly the coating adheres to the foundation metal was also made. A strip of machine steel  $\frac{1}{4}$ " thick by 3" wide was covered with a paste and subjected to the heat of a blow torch for about 4 hours. After cooling it was bent on a 2" radius. The aluminum had alloyed to such an extent that no unprotected steel was exposed by this severe bending. This test brings out one of the very important features of this new method of treatment, viz., that it may be used for treating spots or areas as, for instance, portions which cannot be fired in the usual way, as well as for repair or patch work.

As to the particular materials and proportions, I have found that a good paste is made by mixing 40 grs. of granular aluminum with 25 c. c. of 6 oz. pyroxylin solution. For spraying, the following was worked out for use with a De Vilbiss, type D, spray gun: 40 gm. granular aluminum 20 c. c. 6 oz. pyroxylin solution, 10 c. c. benzol, 5 c. c. amyl acetate.

This mixture sprays well, forms an adherent coating and there is little difficulty in keeping the aluminum in suspension. For dipping I have found that a very fine granular aluminum is preferable. The aluminum powder should be fine enough to pass through a 270 mesh screen to give the best results with the dipping process. When flaked aluminum powder is used in whole or in part the coating thus obtained is not as good as where the granular aluminum powder only is used. As to the degree of fineness of the aluminum granules, I have found that this depends somewhat upon the nature

of the coating desired. For smooth coatings a very fine mesh screen is preferable, while a coarser mesh appears to be better for a heavier and more resistant coating. A mixture of the two is often found desirable.

While I have specified certain materials and proportions thereof which I have found to give very good results, it should be understood that my invention is in no sense limited in this respect. For instance, cellulose acetate might be used instead of cellulose nitrate, although I have not found it to give as good results. One of the reasons for this seems to be that the solvents for cellulose acetate are more hygroscopic than those employed with cellulose nitrate and hence do not evaporate as rapidly. Coatings will not, therefore, dry quickly unless heated, but if subjected to moist atmosphere before solvents have evaporated, there will be a tendency for the coating to absorb moisture and precipitate out the cellulose. Another reason is that at the present time cellulose acetate costs much more than cellulose nitrate. As to the character of the aluminum, I have stated above that the granular or powdered material is preferable to flake aluminum, such as used in aluminum paints, and the reasons seem to be; first, there is less surface exposed and, consequently, less oxide in the metal; second, less solution is required for the mixture; third, the hardened coating is more durable, which is very important if the coated articles are not fired immediately. However, further experience might demonstrate some or all of these conclusions to be erroneous and I therefore wish it understood that my invention is not limited in respect to the particular materials employed or to their proportions or methods of handling except insofar as it is limited by the scope of the claims annexed hereto.

What I claim as new and desire to secure by Letters Patent of the United States is:—

1. The process of protecting metallic articles from oxidation which consists in covering the surface of the article with a mix-

ture of another metal in powdered form and a nitrocellulose binder, and then firing at a temperature which will cause the powdered metal to alloy with the metal of the article.

2. The process of protecting metallic articles from oxidation which consists in covering the surface to be protected with a powdered metal adapted to form an oxidation resisting alloy with the metal of the article, said powdered covering metal being applied at ordinary temperatures in combination with a cellulose derivative binder, and then firing at a temperature which will cause the covering metal to alloy with the metal of the article.

3. The process of protecting metallic articles from oxidation which consists in covering at ordinary temperatures the surface of the article with a mixture of aluminum powder and a liquid consisting of nitrocellulose and a volatile solvent, and then firing at a temperature which will cause the aluminum to alloy with the metal of the article.

4. The process of protecting metallic articles from oxidation which consists in covering the article with a coating composed of aluminum powder and a binder having a cellulose nitrate base, drying the coating, then firing it at a temperature which will cause the aluminum to alloy with the metal of the article.

5. The process of protecting metallic articles from oxidation which consists in covering the articles at ordinary temperatures with a coating composed of aluminum powder and a liquid nitrocellulose binder which wets and firmly adheres to metals at ordinary temperatures and volatilizes at higher temperatures, drying the coating and then firing at a temperature at which the aluminum alloys with the metal of the article, said temperature being above that at which the binder volatilizes.

In witness whereof I have hereunto set my hand this 31st day of March, 1925.

GOODWIN H. HOWE.